

June 17, 1941.

F. L. McENANY

2,246,101

FLOOR COVERING

Filed Jan. 14, 1938



Fig. 1



Fig. 2



Fig. 3



Fig. 4



Fig. 5



Fig. 6



Fig. 7



Fig. 8



Fig. 9



Fig. 10

Frederick Lester McEnany, INVENTOR.

BY *R. F. Miller*

ATTORNEY.

## UNITED STATES PATENT OFFICE

2,246,101

## FLOOR COVERING

Frederick L. McEnany, Bridgeport, Conn., assignor to E. I. du Pont de Nemours & Company, Wilmington, Del., a corporation of Delaware

Application January 14, 1938, Serial No. 185,039

1 Claim. (Cl. 154—49)

This invention relates to an improved composite sheet material. More particularly it relates to an improved sheet material for damp proofing cellar floors and the like, which material simultaneously provides a resilient and wear resistant floor covering.

There is an increasing demand for the conversion of cellar rooms in residences to livable rooms, due to the improved heating methods in use today. Many new homes are so constructed that the cellar is readily adapted to serve as a recreation room or extra living room. In older residences, however, the installation of improved heating equipment results in the waste of cellar space because the floors are often damp and moist and the room is, therefore, unsuitable for use.

It is an object of this invention to provide a novel composite sheet material. It is a further object to provide a floor covering which is damp proof, resilient and wear resistant. Other objects will appear hereinafter.

These objects have been accomplished by constructing a composite sheet material having a metal layer, an intermediate resilient layer, and a top layer of wear resistant material. These three layers may be the only layers present, and may adhere to each other in the order named; or additional layers of material may be added; or one or more of the three named layers may consist of more than one sublayer.

In the accompanying drawing:

Fig. 1 is a perspective view of a portion of a room the floor of which is covered with the novel composite sheet material.

Fig. 2 is a perspective view of one form of the novel composite sheet material the end of which is shown in section.

Figs. 3 to 10 are sections of modifications of the composite sheet material according to the invention.

In order that the invention may be more fully understood, a preferred embodiment thereof will now be described, but it is to be understood that suitable changes may be made from the specific embodiment described without departing from the spirit and scope of the invention as will become more apparent hereinafter.

A layer of non-cellular rubber is coated on one side of a fabric, such, for example, as woven or knitted cloth, and vulcanized thereupon. The vulcanizing is done in a manner well understood by those skilled in the art. There is thus formed a wear resistant layer about  $\frac{1}{8}$  inch in thickness.

A layer of sponge rubber about  $\frac{1}{4}$  inch in thick-

ness is prepared in known manner. Sponge rubber is of a cellular structure as the name implies and possesses excellent resilient characteristics. It may be prepared in a manner described by

5 P. Kohler in Kautschuk, vol. 11, pages 46 to 48 and 69 (1935); or by any of the patented processes as, for example, by the process of U. S. Patent No. 1,877,527, issued September 13, 1932.

The layer of sponge rubber is then cemented to 10 the fabric of the wear resistant layer in the following manner.

There is spread upon the sponge rubber surface an adhesive cement of the following composition:

|                | Parts by weight |
|----------------|-----------------|
| Crepe rubber   | 50              |
| Burgundy pitch | 10              |
| Rosin          | 10              |
| Whiting        | 30              |
| Gasoline       | 100             |

A layer of the same adhesive cement is applied to the fabric surface. The solvent is evaporated from the adhesive cement on the two sheets until the proper degree of tackiness is attained and then the two sheets are placed in contact with their adhesive coated surfaces together. A sheet of copper about .004 inch thick and weighing about one ounce per sq. ft. is cemented to the 25 remaining exposed side of the sponge rubber in the same manner as just described. The composite sheet material in this example is made of strips 54 inches in width and the copper layer combined with the other layers in such manner 30 that it extends three inches beyond the edge of the upper layers on one side and three inches short of the edge of the upper layers on the other side.

In applying the composite sheet material of the 35 invention to a cellar floor or the like, the floor is first dried as thoroughly as possible and a film of adhesive composition such, for example, as that above stated is applied to the floor and a film of the same adhesive is applied to the copper 40 surface of the composite sheet material. When the solvent of the adhesive has evaporated until the proper tackiness has been attained, the sheet material is laid upon the floor and pressed firmly 45 in place. Seams are formed by the offset edges being applied one over the other and adhesively 50 secured in the same manner. It has been found preferable to bend the sheet material and adhere it to the side wall for a short distance above the floor, depending upon existing conditions. 55 In this manner, the damp proofing of the cellar

may be made more effective. The sheet material produced as described is flexible to a remarkable degree and can be bent, folded and worked with ease.

Figure 1 of the drawing shows a corner of a room, the floor of which has been covered with a composite sheet material such as above described. In this figure, 8 is a brick wall and 9 is a cement floor. It is to be understood, however, that the floor may be of wood or other structural material. Eleven is the solid rubber tread and 13 is the fabric to which it is vulcanized. Eleven and 13 together form the wear resistant tread layer. Sponge rubber resilient layer 15 is attached to fabric 13 by cement 14, and is attached to waterproof copper layer 19 by cement 16. The waterproof copper layer is attached to the floor 9 and side walls 8 by means of cement 7, the composite sheet material being bent at right angles to extend upward along the walls as shown.

Fig. 2 shows a portion of a strip of the composite sheet material with the metal waterproof layer offset from the other layers for the purpose of forming a seam as has been described above.

It is evident that changes may be made in the composition of the various layers and that additional layers of material may also be added without departing from the spirit of the invention. While copper is preferred for the waterproofing layer, other non-rusting metals such as aluminum, tin, zinc, and brass may be used. While sponge rubber is preferred for the resilient layer, other materials such as sponge neoprene, cork, or paper may be used, although, in general, these other materials have not been found to be as satisfactory as sponge rubber. The preferred material for the wear resistant tread layer is solid rubber of non-cellular structure, but neoprene, carpet, or linoleum may be substituted therefor. In fact any wear resistant tread material known in the art may be used for this layer. Where a bond between rubber and another material is to be made, this may be accomplished by vulcanizing the rubber to said other material or by the use of a suitable cement. While the specific example has disclosed the composite sheet material cemented to the floor, it will be satisfactory in some instances to lay the sheet material upon the floor without cementing it thereto. Instead of forming a seam by offset edges as disclosed in the specific example, the edges of the strips of composite sheet material may be flush and the seam may be formed by cementing, soldering, welding or otherwise securing a narrow strip of metal over the abutting edges of the waterproof sheet of metal.

In order that the invention may be better understood, Figs. 3 to 10 have been included to illustrate several modifications of the invention.

In Fig. 3, the solid rubber tread layer 31 is vulcanized to fabric layer 33 and sponge rubber resilient layer 35 is vulcanized to fabric layer 33. Waterproof metal layer 39 is cemented to sponge rubber layer 35 by cement 36.

In Fig. 4, solid rubber tread layer 41 is attached to fabric layer 43 by means of cement 42. Sponge rubber layer 45 is vulcanized to fabric layer 43, and waterproof metal layer 49 is cemented to sponge rubber layer 45 by means of cement 46.

In Fig. 5, the solid rubber layer 51, fabric layer 53, sponge rubber layer 55 and waterproof metal layer 59 are cemented together in the order named by cement layers 52, 54, and 56.

Fig. 6 shows a wear resistant tread layer of linoleum 61 attached to resilient layer 65 by means of cement 62 and waterproof metal layer 69 attached to resilient layer 65 by means of cement 66.

Fig. 7 shows resistant tread layers of linoleum 71 attached to resilient layer 75 by means of cement layer 72. A layer of craft paper 77 attached to resilient layer 75 by means of cement layer 76 and waterproof metal layer 79 attached to craft paper 77 by means of sisal fibre cement 78.

In Fig. 8, carpet layer 81 is attached to resilient layer 85 by means of cement 82 and the resilient layer is in turn attached to waterproof layer 89 by means of cement 86.

Fig. 9 shows resilient sponge rubber layer 95 vulcanized to carpet layer 91 and attached to waterproof metal layer 99 by cement 96.

Fig. 10 shows solid rubber tread layer 101 and resilient sponge rubber layer 105 vulcanized to opposite sides of cloth layer 103. Waterproof metal layer 109 is attached to craft paper layer 107 by sisal fibre cement 108. Craft paper 107 is attached to sponge rubber layer 105 by a cement 106.

Other modifications of the invention will readily suggest themselves to those skilled in the art.

The cement used in attaching the various layers to each other may be that disclosed above in the detailed specific example, it may consist of the ingredients of the detailed specific examples compounded in other proportions than those therein disclosed, or any other suitable cement or adhesive may be used, such, for example, as marine glue, asphalt, adhesive prepared from cellulose derivatives and the like.

It is sometimes desirable to use an intermediate layer of paper between the metal layer and the resilient layer to improve adhesion between such layers. While any layer of paper may be used, it has been found especially desirable to use for this purpose a paper-metal combination which is obtained commercially under the name "Copper Armored Sisal Craft."

It is not intended to limit the invention by the dimensions of any or all of the layers to those recited in the detailed specific example. The metal layer may vary from a thin foil of .001 inch or more in thickness to a sheet of .100 inch or more in thickness, but it has been found that a thickness of .004 inch is most satisfactory from the standpoint of economy, flexibility and protection against dampness. Likewise, the resilient layer which is preferably of sponge rubber may vary from .025 inch to one inch or more, although, in general, it has been found that this layer should be at least .25 inch to obtain a desirable resilience. The tread surface layer may be of any thickness consistent with flexibility. While the finished sheet material may be of any width, it has been found that it is more easily handled in strips from 36 to 54 inches wide.

The composite sheet material of this invention is of great usefulness in the conversion of damp cellar rooms to inhabitable rooms by being placed on the floor thereof as has been described. It is also suitable for application to all types of floor such as those in garages, workshops, cottages and the like. It provides a means for damp-proofing floors without the necessity of resorting to costly and laborious reconstruction and at the same time provides a floor covering which may be used without the laying of a separate tread material.

The composite sheet material of this invention

may also be used for heat and sound insulation, as, for example, upon the floor of automobiles, railway coaches and the like.

It is apparent that many widely different embodiments of this invention may be made without departing from the spirit and scope thereof; and, therefore, it is not intended to be limited except as indicated in the appended claim.

I claim:

In a floor covering highly flexible strips of 10 laminated material which form an assembled unitary structure for application as a damp-proofing floor covering and which is capable of

being folded and of being bent at right angles to continue the covering from the floor to the side walls, said strips comprising a tread layer of non-cellular rubber, a layer of fabric attached to 5 said rubber layer, a bottom layer of thin copper foil, a sponge rubber layer which is of substantially greater thickness than the above mentioned other layers and which is positioned between said fabric layer and layer of copper foil, and a layer of cement between said sponge rubber layer and said layer of copper foil.

FREDERICK L. McENANY.